

melted 5  
 pitch 2 1/2  
 acid 8 lbs  
 18 oz

251,054

# UNITED STATES PATENT OFFICE.

EUGENE JONES, OF GOLD HILL, NEVADA.

## PAINT COMPOUND FOR METALLIC SURFACES.

SPECIFICATION forming part of Letters Patent No. 251,054, dated December 20, 1881.

Application filed July 18, 1881. (No specimen.s.)

*To all whom it may concern:*

Be it known that I, EUGENE JONES, of Gold Hill, Storey county, State of Nevada, have invented a Compound for the Protection of Wire 5 Ropes, &c.; and I do hereby declare the following to be a full, clear, and exact description thereof.

My invention relates to a compound which is used for covering wire ropes such as are employed for mining purposes, rigging of ships, cable-railroads, and in other places; and it can also be applied to the bottoms of ships, water-pipes, and other metallic surfaces.

The object of my compound is to prevent corrod ing or crystallizing of the article on which it is placed either when used under water or exposed to the atmosphere.

In manufacturing my compound I take thirty (30) gallons of tar, which has been previously heated or parboiled, and after placing it in a suitable receptacle, heat it, and then introduce the following ingredients—to wit: five (5) gallons melted tallow, two and one-half (2 1/2) gallons black pitch, and eight (8) pounds rosin. 25 After the whole has been thoroughly mixed and heated to a boiling-point I pour into the mixture eighteen (18) ounces of gallic acid.

I do not materially change the above pro-

portions, whether making larger or smaller quantities of the compound.

I usually apply to flat surfaces with a brush or similar article; but in case of cables or other surfaces which are to be used in hot mining-shafts or under water they are covered by the mixture when in a boiling-hot condition.

For the sake of economy I sometimes substitute tanner's bark for gallic acid.

I am aware tar, tallow, pitch, rosin, tanning material, and the like have been used as ingredients in compositions for coating materials; but I am not aware that the herein-claimed compound, as an entirety, has been used, and in the proportions set forth.

Having thus described my invention, what I claim as new, and desire to secure by Letters Patent, is—

A compound for covering metallic surfaces, consisting of tar, tallow, black pitch, rosin, and gallic acid, in about the proportions and for the purpose herein described.

In witness whereof I have hereunto set my hand.

EUGENE JONES.

Witnesses:

FRANK A. BROOKS,  
JOSEPH A. BAYLESS.